

## UNITED STATES PATENT OFFICE

2,488,588

## TREATMENT OF TEXTILE MATERIALS

Camille Dreyfus, New York, N. Y., and George W. Seymour and George C. Ward, Cumberland, Md., assignors to Celanese Corporation of America, a corporation of Delaware.

No Drawing. Application July 11, 1945,  
Serial No. 604,502

5 Claims. (Cl. 117—138)

1

This invention relates to the treatment of textile materials and relates more particularly to a novel process for the treatment of textile materials in fabric form made of or containing filaments or fibers of a non-thermoplastic character to effect a substantial improvement in the heat resistance and ironing qualities of said textile materials.

An object of this invention is to provide an improved process for the treatment of textile materials having a basis of non-thermoplastic artificial or naturally-occurring filaments or fibers to impart improved ironing and heat-resisting qualities thereto.

Another object of this invention is to raise the safe-ironing temperature of non-thermoplastic textile materials whereby scorching or other undesirable effects produced by the application of too hot an iron thereto may be substantially eliminated.

Other objects of this invention will appear from the following detailed description.

Fabrics woven of yarns having a basis of filaments or fibers of non-thermoplastic naturally-occurring or artificial materials may be ironed at temperatures substantially higher than textile materials having a basis of thermoplastic filaments or fibers. Thus, thermoplastic materials may be ironed safely at temperatures up to about 220° C. while non-thermoplastic materials such as cotton, for example, may be safely ironed at temperatures up to about 240 to 250° C. While there is no danger of melting or coalescing the non-thermoplastic textile materials when ironed at temperatures appreciably above 250° C., the materials may be scorched with the result that the strength and appearance of said materials are permanently impaired. The elimination of scorching or other undesirable effect due to the use of excessively high ironing temperatures by treating said materials so as to raise substantially the temperature at which ironing of these materials may be safely conducted would be highly advantageous.

We have now found that the resistance of fabrics made of or containing non-thermoplastic textile materials to scorching at higher ironing temperatures may be substantially increased by subjecting said materials to treatment with an aqueous solution of boric acid.

The aqueous boric acid solution employed may contain from 1 to 15% by weight of boric acid and may be applied by padding, dipping or rinsing the textile material in said solution. Any boric acid solution in excess of the amount de-

sired to be permitted to remain on the textile material may be removed by passing the treated material through squeeze rolls and the textile material, with the desired quantity of boric acid remaining thereon, may then be dried in any convenient manner. The drying may be effected by passing the fabric through a suitable chamber through which the heated air at a temperature of 85 to 110° C. is circulated or by passing the fabric over heated drums or cans. In this way, from 1 to 15% by weight of boric acid on the weight of the fabric undergoing treatment may be uniformly applied thereto.

After drying, the fabric is then preferably subjected to hot calendering or mangling or decatizing. When the fabric is subjected to mangling or hot calendering, temperatures of 110 to 150° C. and pressures of 2000 to 8000 pounds per square inch are usually employed.

20 The decatizing treatment that may be used consists in winding the fabric on to a perforated metal drum with a heavy cotton blanket or apron so that a layer of the cotton blanket or apron alternates with each layer of the fabric. Steam at 25 a pressure of the order of 10 pounds per square inch or more is then passed through the fabric for 3 to 5 minutes, whereby the temperature of the fabric is raised to 95 to 110° C., thereupon the steam is shut off and vacuum is applied to cool the fabric and remove any condensed water present.

30 Fabrics made of or containing non-thermoplastic filaments or fibers and treated in accordance with our novel process may then be ironed at substantially increased temperatures as compared to untreated fabrics without undergoing scorching or changes detrimentally affecting the fabrics undergoing ironing.

40 As examples of non-thermoplastic textile materials of which the fabrics treated in accordance with our novel process may be formed, there may be mentioned cotton, wool, regenerated cellulose prepared by the viscose process, as well as regenerated cellulose obtained by the saponification of filaments or fibers having a basis of cellulose acetate or other organic derivative of cellulose especially strong yarns made by the saponification of yarns of cellulose acetate that have been 45 stretched while in a softened condition. The fabric treated may contain two or more of any of the above non-thermoplastic fibers.

50 In order further to illustrate our invention but without being limited thereto the following examples are given:

## Example I

A fabric of white cotton cheesecloth is padded with a 5% aqueous boric acid solution at a temperature of 38° C., the fabric being permitted to retain about 100% by weight of the solution. The padded fabric is then dried with heated air at a temperature of 110° C. in a suitable drying chamber and then decatized. When the treated fabric is subjected to the action of a stationary hand iron at a temperature of 280° C. for 10 seconds, the material remains entirely unaffected, while an untreated cotton material subjected to the same test scorches with the production of a deep brown color where the material was in contact with the heated surface of the iron.

## Example II

A fabric woven of strong regenerated cellulose yarns prepared by completely saponifying cellulose acetate yarns that have been stretched while in a softened state with a suitable saponifying agent is padded with a 5% aqueous solution of boric acid at 38° C. and the fabric is allowed to retain 100% by weight of the solution. The fabric is then dried with air heated at about 100° C. and decatized. When the treated fabric is subjected to the 10 second stationary iron test, the testing iron being at a temperature of 270° C., no change in the physical appearance of the fabric tested is observed as a result of this test, while untreated fabric undergoing this test becomes quite scorched at the point of contact with the iron.

## Example III

A taffeta fabric woven of regenerated cellulose yarns prepared by the viscose process is padded with a 5% aqueous solution of boric acid at 38° C. The fabric is allowed to retain 100% by weight of the solution and is then dried with air heated at 100° C. and decatized. When a hand iron heated to 240° C. is allowed to stand on a treated fabric for 10 seconds, no change in the physical appearance of the fabric is observed. The untreated fabric undergoing this test becomes noticeably scorched.

Other methods of applying the boric acid may be used. Thus garments made of fabrics comprising a non-thermoplastic fiber, after they are laundered either at home or in commercial laundries, may be given a final rinse in boric acid solution and then subjected to hydro-extracting or vacuum-extracting and then mangled. Thereupon the garments may be ironed with a quite hot iron without any danger of scorching.

It is to be understood that the foregoing detailed description is given merely by way of illustration and that many variations may be made therein without departing from the spirit of our invention.

Having described our invention what we desire to secure by Letters Patent is:

1. Process for improving the ironing and heat-resisting properties of textile materials comprising filaments and fibers having a basis of a non-thermoplastic textile material, which comprises

applying a solution of boric acid to said materials, drying the treated materials and then subjecting them to a heat treatment at a temperature of at least 110° C. under a pressure at least 2000 lbs. per square inch.

2. Process for improving the ironing and heat-resisting properties of textile materials comprising filaments and fibers having a basis of a non-thermoplastic textile material, which comprises applying a 1 to 15% aqueous solution of boric acid to said materials, drying the treated materials and then subjecting the dried materials to a heat treatment at a temperature of 110 to 150° C. and a pressure of 2000 to 8000 pounds per square inch.

3. Process for improving the ironing and heat-resisting properties of textile materials comprising filaments and fibers having a basis of cotton, which comprises applying a 1 to 15% aqueous solution of boric acid to said materials, drying the treated materials and then subjecting the dried materials to a heat treatment at a temperature of 110 to 150° C. and a pressure of 2000 to 8000 pounds per square inch.

4. Process for improving the ironing and heat-resisting properties of textile materials comprising filaments and fibers having a basis of regenerated cellulose, which comprises applying a 1 to 15% aqueous solution of boric acid to said materials, drying the treated materials and then subjecting the dried materials to a heat treatment at a temperature of 110 to 150° C. and a pressure of 2000 to 8000 pounds per square inch.

5. Process for improving the ironing and heat-resisting properties of textile materials comprising filaments and fibers having a basis of wool, which comprises applying a 1 to 15% aqueous solution of boric acid to said materials, drying the treated materials and then subjecting the dried materials to a heat treatment at a temperature of 110 to 150° C. and a pressure of 2000 to 8000 pounds per square inch.

CAMILLE DREYFUS.  
GEORGE W. SEYMOUR.  
GEORGE C. WARD.

## REFERENCES CITED

The following references are of record in the file of this patent:

## UNITED STATES PATENTS

| Number    | Name            | Date          |
|-----------|-----------------|---------------|
| 865,033   | Haley           | Sept. 3, 1907 |
| 1,501,895 | Andrus          | July 22, 1924 |
| 1,738,976 | Vivas           | Dec. 10, 1929 |
| 2,072,253 | Ellis           | Mar. 2, 1937  |
| 2,185,695 | Oliver          | Jan. 2, 1940  |
| 2,300,982 | Slagboom et al. | Nov. 3, 1942  |
| 2,326,605 | Bass et al.     | Aug. 10, 1943 |

## OTHER REFERENCES

Leatherman Farmers' Bulletin No. 1786, U. S. Dept. Agriculture, Dec. 1937.  
65 Tweedie et al., American Dyestuff Reporter, pp. 427-428, Sept. 27, 1943.